# EUROPEAN PATENT SPECIFICATION

(11) **EP 1 492 654 B1**
(45) Date of publication and mention of the grant of the patent: **31.10.2007**
(21) Application number: 03719012.1
(22) Date of filing: 27.03.2003
(51) Int. Cl.: B27K 3/30

(54) **Use of an aqueous solution of one or more bifluorides for improving the drying process of green wood**
Verwendung einer wässrigen Lösung mit einem oder mehreren Bifluoriden zur Verbesserung des Trocknungsprozesses von Frischholz
Utilisation d'une solution aqueuse d'un ou plusieurs bifluorides pour améliorer le procédé de séchage de bois vert

(30) Priority: 29.03.2002 NL 1020280
(43) Date of publication of application: 05.01.2005
(73) Proprietor: NIJMAN WOOD MODIFICATION TRADING COMPANY LTD., Dublin 1 (IE)
(72) Inventor: NIJMAN, Henrikus, Franciscus, Maria, NL-2264 TG Leidschendam (NL)
(74) Representative: van Assen, Jan Willem Bernard
(86) International application number: PCT/IB2003/001794
(87) International publication number: WO 2003/082534

(56) References cited:
- EP-A- 0 139 142
- BE-A- 449 703
- DE-C- 749 183
- NL-C- 1 004 556
- DATABASE WPI Section Ch, Week 199014 Derwent Publications Ltd., London, GB; Class C03, AN 1990-106135 XP002222265 & SU 1 509 252 A (SENEZH WOOD PRESERV), 23 September 1989 (1989-09-23)

## Description

The invention relates to the use of an aqueous solution of one or more bifluorides for improving the drying process of green wood by wetting the green wood with an aqueous solution containing one or more bifluorides by immersion or spraying for at least 3 minutes.

With respect to the previous, from Dutch Patent No. 1004556 a method is known for the treatment of wood, by which the bifluoride solution contains 8 - 32 weights% of both potassium and ammonium bifluoride in a weights proportion of the potassium to the ammonium salt between 13 : 7 and 2 : 3. The treatment known from Dutch Patent No. 1004556 has as purpose the improvement of the moisture regulating properties of the wood or the products made from that.

A problem with green wood is that it cracks by drying too fast, with the result that per unity of volume less useful products can be made from that.

From John H. Perry, Chemical Engineer's Handbook, Second Edition, McGraw Hill Book Company, New York, p. 1509, for the solution of this problem a lumber dryer is known, by which wood is dried at elevated temperature under controlled relative humidity with heated air.

The said dryer is called "Tiemann lumber dryer" and a cross - section of this dryer is shown as Figure 9 on p. 1509 of the previously mentioned publication.

Self - evidently drying with heated air under controlled relative humidity is quite expensive, more especially because of the heat needed.

From JP - A - 07 - 314409 (Chem. Abs. 124:149094v) another method for impregnation of wood without the necessity of pre - drying, by which cracking of the wood is prevented, is known.

First the "green" wood is impregnated with an organic solvent, compatible with wood and miscible with water. After extraction and replacement of most of the water with organic solvent, subsequently the wood is impregnated with preserving agents soluble in the organic solvent.

Self - evidently this impregnation is expensive and it can be questioned whether the organic impregnation agents used are sufficiently harmless for the environment.

According to the invention the wood is immersed or sprayed on all sides during at least 3 minutes with the bifluoride solution.

With the treatment according to the invention one is not limited to the mixture of potassium and ammonium bifluoride of Dutch Patent No. 1004556, but eventually other bifluorides with a high solubility in water could be used too.

Discovered was namely that during the very short all sided wetting of the wood, the bifluoride penetrates sufficiently deep in the outer layers of the wood for improving the drying process in such an extent, that heated drying with risk of cracking becomes superfluous.

In this case the wetting of the wood has to be all sided.

During a wetting of the wood, the bifluoride ion (FHF') from the mixed bifluoride solution penetrates very quickly in the outer layers of the wood.

As before mentioned, the invention is based on the discovery that when the amount of water capacity is greater than the amount of water present in completely dry wood, the chemisorption of FHF' on cellulose is as if it were catalysed and therewith enters in a lasting bond with cellulose.

According to the invention one can use also in addition to the mixture of potassium and ammonium fluoride mentioned in Dutch Patent No. 1004556 another alkali bifluoride, and one can use the bifluorides separately also, provided that with wood is satisfied on the concentration of 8 - 32 weights%.

A preferred wetting solution is the solution mentioned in Dutch Patent No. 1004556 of potassium and ammonium bifluoride by which the weights proportion between both bifluorides is between 13 : 7 and 2 : 3.

In addition to the before mentioned alkali bifluorides, it is possible also to use one or more other bifluorides, which are fairly soluble, zinc bifluoride for instance is conceivable.

Self - evidently the wetting solution may contain other soluble metal salts in addition to one or more alkali bifluorides and/or zinc bifluoride.

Arbitrarily in the sense of the invention it can be postulated that green wood is wood with a moisture content above 8 weigts%.

As consequence of the treatment through all sided wetting with bifluoride solution according to the invention, the moisture content in the outer layers of the wood increases during a short time with several percents. During drying the moisture content in the outer layers of the treated wood falls rather quickly to somewhat below the initial moisture content preceding the immersion treatment.

The consequence of the wood treatment is that the outer layers with chemisorbed bifluoride dry better with conservation of the moisture regulation properties of the wood.

Preferably the all sided wetting can take place trough immersion on lath.

It is noted that in Dutch Patent No. 1004556 on p. 5 lines 26 and 27 it is mentioned that if necessary wooden components eventually can already be placed on lath during the immersion in the solution of the combined bifluorides.

However components are wooden parts, which as a rule are made from wood pre - dried in the wood producing countries.

The method according to the invention now can advantageously be applied on "green" wood.

As mentioned before, it has been discovered that amounts of water greater than the equilibrium concentration in dry wood accelerate greatly the penetration of the FHF'.

With "green" wood are meant tree - trunks of just felled trees, whether or not stripped of their bark or boards or beams sawed there from a short time after felling.

Self - evidently this has great consequences for the wood industry, wood can now namely almost simultaneously be treated with bifluoride solution and dried.

The method according to the invention can advantageously be applied as follows.

One uses a bifluoride solution with a weights concentration between 8 and 15 weights% for wood with a moisture content between 10 and 35%; for more humid wood one uses a bifluoride solution with a higher weights concentration. Therefore a bifluoride solution with a weights concentration between 15 and 32 weights% is used for wood with a moisture content between 35 and 60%.

According to a preferred method and equipment, with which green wood or incompletely dry wood can be treated, is wood as with the known quick dry installation stacked in such a way on transport vehicles, that warm drying air can flow through and along the tree-trunks to be dried, one elaborates more or less on the here before mentioned "Tiemann's lumber dryer".

With the method and equipment according to the invention, the wood is first stacked on lath in a transport container.

The equipment includes in addition to the transport container an immersion vessel with agitation means for improvement of the all sided rinsing of the wood with the bifluoride solution and means for bringing in - and out - of the transport container in the immersion vessel.

After immersion of the wood in the immersion vessel, the wood is lifted out of the bifluoride bath and is left over to draining in the immersion vessel.

After draining the wood is ready for transport in the transport container and dries due to the improved moisture regulating properties already during the transport.

The immersion vessel is hereby provided with dosing means for bifluoride solution.

The product obtained by means of the pre - treatment is through that better suited for manufacture of formed objects or the formed objects possess better properties.

Most probable the improvement of the properties is due to chemisorption of FHF' ions on cellulose, whereon follows complete modification.

Continuing with the obtained improved properties of the treated cellulose, it is now proposed to pre - treat with bifluoride wood powder and possibly other fairly fine products, such as cotton linters and flax fluffy after which it is the intention to convert the treated material further to useful products.

Other fairly fine products are straw, broken flax stalks and cotton fiber.

The invention relates also to wood modified with bifluoride solution or wooden products made thereof.

As mentioned before the invention relates in principle to improvement of the properties of cellulose treated with bifluoride and/or formed objects hereof.

With treated cellulose in the meaning of the invention is meant also wood powder, cotton linters, flax fluffy and like materials such as whether or not grinded straw or bagasse.

The invention elaborates on model experiments performed as a result of Dutch Patent No. 1004556 in order to imitate the effect of relatively small amounts of bifluoride on the good moisture regulation of a wood treated with potassium and ammonium bifluoride and to find out the probably cause thereof.

Most probably the improvement of the properties is due to chemisorption of FHF' ions on cellulose.

The invention is illustrated now with four examples and a graph with respect to the penetration depth in wood, and a graph with respect to the moisture regulation behaviour of treated cellulose.

With respect to the examples and the graph of the penetration in wood it is firstly remarked that the moisture content of wood is determined with the formula $\frac{{A}_{x} - B}{{A}_{100}} \times 100 % ,$ wherein
Aₓ weight of wood with a certain moisture content
A₁₀₀ weight of wood which is completely moist,
B weight of wood which is completely dry.

The weight of completely dry wood is determined through drying this during 24 hours at 110°C.

Ax is the weight of wood with a moisture content between 0 and 100%.

Further it is remarked with respect to the penetration depth of bifluorides in wood that this is determined with zirconyl - alizarine S reagent (J. H. de Boer, Chemisch Weekblad 21, 404 (1924)).

Firstly the wood treated with bifluoride solution is sawed off transversely to the penetration depth and subsequently thinly sprayed with zirconyl- alizarine S reagent. On the spot, or penetration depth, where chemisorbed bifluoride is present, this reacts with the red - violet zirconyl - alizarine S. By the reaction with the bifluoride, the red - violet colour is changed in pale yellow ( that of the liberated alizarine sulfonic acid) because of the formation of the colourless bivalent zirconium hexafluoride ion ZrF₆".

As cellulose is the most important constituent of wood, the following experiments with cellulose were performed in order to demonstrate the changes in adsorption behaviour of wood.

With the experiments with cellulose six A4 sheets bleached softwood cellulose pulp were respectively immersed in bifluoride solution and demineralised water, each three pieces.

The cellulose pulp sheets weighted each about 50 grams.

The 10 seconds immersion time is beforehand determined as the maximal immersion time before the specimen disintegrates through the action of moisture.

After immersion the specimen was dried at the air during 1 minute and subsequently fastened on a weighing device in a climatic room. Subsequently, the cellulose sheet was equilibrated with the environment during 8 hours, at 23°C at 50% RH ( relative humidity) before starting the experiment.

With the three experiments of cellulose treated with bifluoride and the three experiments treated with demineralised water, the cellulose sheet was first exposed to an air atmosphere of 23°C with a RH of 85% during about 8 hours and subsequently to an air atmosphere of 23°C with a RH of 35% during about 7 hours.

The weights of all the six specimens at the start of the individual experiments are about 50 grams, the weights of the three cellulose sheets treated with bifluoride gradually increase with about 8 grams of water, at lowering of the RH to 35%, the absorbed water rather steeply disappears except to about 2 grams.

With a cellulose sheet treated with demineralised water only, the weight increases much less than with a specimen pre - treated with bifluoride. Herewith the increase in weight is about 1,5 grams only and returns with RH reduction much less steeply to about the weight at the start of the experiment.

Prolonged experience with wood treated with bifluoride solution has shown that this through the changed water absorbtion behaviour, which is supported by the fast absorption and desorption of water with change of RH of cellulose, has improved properties with respect to wood moisture regulation.

The moisture absorption behaviour of wood changed through the treatment with bifluoride solution extends also to wood powder, wood pulp or other disintegrated products from materials with a high cellulose content.

In addition to the above mentioned concept of the improved moisture regulation of wood or disintegrated cellulose containing materials, the invention relates as mentioned before to the discovery that the penetration of aqueous bifluoride solution is if it were catalysed by moisture.

Because of this advantage one has not to impregnate under pressure or vacuum a wood preservation solution in order to obtain a sufficient penetration depth.

## Claims

1. The use of an aqueous solution of one or more bifluorides for improving the drying process of green wood, by wetting said green wood with said solution by immersion or spraying for at least 3 minutes.

2. Use according to claim 1, **characterized in that**, one immerses the green wood on slat.

3. Use according to claim 1, **characterized in that**, one sprays the green wood all sided.

4. Use according to claims 1 - 3, **characterized in that**, one uses for the wetting an aqueous solution which contains one or more alkali bifluorides.

5. Use according to claim 4, **characterized in that**, the bifluoride solution contains potassium and ammonium bifluoride, in which the weights ratio between both bifluorides is between 13 : 7 and 2 : 3.

6. Use according to anyone of claims 1 - 5, **characterized in that**, the bifluoride solution contains one or more other bifluorides as for instance zinc bifluoride, and if necessary other soluble metal salts.

7. Use according to claim 5, **characterized in that** one applies a mixed bifluoride solution with a weight concentration between 8 and 15 weight % on green wood with a moisture content between 10 and 35 % and a mixed bifluoride solution with a weight concentration between 15 and 32 weight % on green wood with a moisture content between 35 and 60 %.

8. Use according to claims 1, 2, 4, 5, 6, or 7, wherein airily stacked green wood is placed on a transport container, subsequently immersed on all sides in aqueous bifluoride solution and after draining, and it desired, drying, transported.

## Patentansprüche

1. Verwendung einer wässrigen Lösung aus einem oder mehreren Bifluoriden zur Verbesserung des Trocknungsprozesses von Frischholz durch Benetzen dieses Frischholzes mit dieser Lösung durch Eintauchen oder Besprühen für zumindest drei Minuten.

2. Verwendung gemäß Anspruch 1, **dadurch gekennzeichnet, dass** man das Frischholz auf einer Leiste eintaucht.

3. Verwendung gemäß Anspruch 1, **dadurch gekennzeichnet, dass** man das Frischholz auf allen Seiten einsprüht.

4. Verwendung gemäß Ansprüchen 1-3, **dadurch gekennzeichnet, dass** man für die Benetzung eine wässrige Lösung verwendet, die ein oder mehrere Alkalibifluoride enthält.

5. Verwendung gemäß Anspruch 4, **dadurch gekennzeichnet, dass** die Bifluoridlösung Kalium- und Ammoniumbifluorid enthält, wobei das Gewichtsverhältnis zwischen beiden Bifluoriden zwischen 13:7 und 2:3 ist.

6. Verwendung gemäß einem der Ansprüche 1-5, **dadurch gekennzeichnet, dass** die Bifluoridlösung ein oder mehrere andere Bifluoride, wie zum Beispiel Zinkbifluorid, sowie falls notwendig andere lösliche Metallsalze enthält.

7. Verwendung gemäß Anspruch 5, **dadurch gekennzeichnet, dass** man eine gemischte Bifluoridlösung mit einer Gewichtskonzentration zwischen 8 und 15 Gewichts-% auf Frischholz mit einem Feuchtigkeitsgehalt zwischen 10 und 35 %, und eine gemischte Bifluoridlösung mit einer Gewichtskonzentration zwischen 15 und 32 Gewichts-% auf Frischholz mit einem Feuchtigkeitsgehalt zwischen 35 und 60 % anwendet.

8. Verwendung gemäß den Ansprüchen 1, 2, 4, 5, 6 oder 7, wobei luftig aufgestapeltes Frischholz auf einem Transportbehälter angeordnet wird, anschließend auf allen Seiten in wässrige Bifluoridlösung eingetaucht wird und nach dem Ablaufen, und falls erwünscht dem Trocknen, transportiert wird.

## Revendications

1. Utilisation d'une solution aqueuse d'un ou plusieurs bifluorures pour améliorer le séchage du bois vert en humidifiant ledit bois vert au moyen de ladite solution par immersion ou pulvérisation pendant au moins trois minutes.

2. Utilisation selon la revendication 1 **caractérisée en ce que** l'immersion du bois vert s'effectue sur lames.

3. Utilisation selon la revendication 1 **caractérisée en ce que** l'on effectue la pulvérisation sur toutes les faces du bois vert.

4. Utilisation selon l'une des revendications 1 à 3 **caractérisée en ce que** l'on utilise pour l'humidification une solution aqueuse contenant un ou plusieurs bifluorures alcalins.

5. Utilisation selon la revendication 4 **caractérisée en ce que** la solution de bifluorure contient du bifluorure de potassium et d'ammonium dans lequel le rapport en poids entre les deux bifluorures est compris entre 13/7 et 2/3.

6. Utilisation selon l'une quelconque des revendications 1 à 5 **caractérisée en ce que** la solution de bifluorure contient un ou plusieurs autres bifluorures parmi lesquels par exemple du bifluorure de zinc, et le cas échéant d'autres sels métalliques sollubles.

7. Utilisation selon la revendication 5 **caractérisée en ce que** l'on met en oeuvre un mélange d'une solution de bifluorure présentant une concentration pondérale de 8 à 15 % en poids du bois vert et une teneur en humidité de 10 à 35 %, avec une solution de bifluorure présentant une concentration pondérale de 15 à 32 % en poids du bois vert et une teneur en humidité de 35 à 60 %.

8. Utilisation selon la revendication 1, 2, 4, 5, 6 ou 7 suivant laquelle du bois vert est empilé à l'air libre et placé sur un réceptacle de transport puis immergé sur toutes ses faces dans une solution de bifluorure aqueuse avant d'être transporté après égouttage suivi d'un séchage éventuel.
